

## UNITED STATES PATENT OFFICE

2,278,725

## MAGNESIUM BASE ALLOY

John C. McDonald, Midland, Mich., assignor to  
 The Dow Chemical Company, Midland, Mich.,  
 a corporation of Michigan

No Drawing. Application October 4, 1940,  
 Serial No. 359,680

4 Claims. (Cl. 75—168)

The invention relates to a magnesium base alloy. It more particularly concerns an alloy of this nature having improved physical properties such as high yield and tensile strengths.

Commercially pure magnesium has been used only to a limited extent as a structural material because of its relatively low strength properties, although its light weight is a highly desirable characteristic for making castings, forgings and other structural forms.

It is, therefore, the principal object of the invention to provide an alloy of magnesium which utilizes the light weight characteristic of magnesium and, at the same time, possesses superior strength properties, rendering it useful for making castings, forgings, and the like, wherein light weight is oftentimes highly desirable.

Other objects and advantages of the invention will be apparent as the description of the invention proceeds.

My invention resides in the discovery that a magnesium base alloy composed of from 0.01 to 3.0 per cent palladium, the balance being substantially all magnesium, possesses the aforementioned properties to a marked degree. The term "magnesium" used herein and in the appended claims is intended to include magnesium containing the ordinary impurities that are found in the commercially pure metal, such as traces of iron, copper, nickel, and silicon. While the properties of high tensile and yield strengths are manifest over the entire range of composition indicated, in general it has been found that the preferred combination of properties such as the most desirable yield strength, coupled with correspondingly high tensile strength is found in those alloys containing from about 0.1 to 2.0 per cent palladium. A preferred alloy having the most desirable combination of yield strength and tensile strength in both the annealed and cold rolled state is one containing about 0.3 per cent palladium.

The following table which lists some of the properties of rolled sheet metal made from my new binary alloy and compares these properties with those of commercially pure magnesium, illustrates the improvement in yield strength and tensile strength of my new alloy over that of the commercially obtainable magnesium. The magnesium used in preparing the new alloy and for

the purposes of comparison was obtained by subliming commercially available magnesium.

Table

| 5  | Nominal composition in percent (magnesium—remainder) Pd | Annealed                       |                                  | Cold rolled                    |                                  |
|----|---------------------------------------------------------|--------------------------------|----------------------------------|--------------------------------|----------------------------------|
|    |                                                         | Yield strength in lbs./sq. in. | Tensile strength in lbs./sq. in. | Yield strength in lbs./sq. in. | Tensile strength in lbs./sq. in. |
| 10 | -----                                                   | 7,000                          | 25,000                           | 14,000                         | 25,000                           |
|    | 0.09                                                    | 17,000                         | 30,000                           | 21,000                         | 29,000                           |
|    | 0.30                                                    | 17,000                         | 30,000                           | 24,000                         | 31,000                           |
|    | 1.00                                                    | 18,000                         | 31,000                           | 23,000                         | 30,000                           |

The properties set forth above under the term "annealed" were obtained by first rolling the specimens at a temperature between 600° and 700° F. and thereafter annealing them at various temperatures through a range of from 400° to 800° F. The properties selected for the table were those of the annealed specimens showing the maximum ductility or formability as measured by the per cent elongation. The properties set forth under the term "cold rolled" were obtained by subjecting specimens which had been first hot rolled at temperatures of from 600° to 700° F. to additional rolling in the cold state. The properties selected for the table were those of the cold rolled specimens which showed the highest tensile and yield strength, while having at least a 1 per cent elongation in 2 inches.

A comparison of the properties listed in the table shows that the yield strength and tensile strength of the new alloy are markedly superior to similar properties of sublimed magnesium in both the annealed and the cold rolled state. This improvement is exhibited throughout the range of composition indicated.

40 The new alloy will be found to be most useful for making castings, extruded forms, and the like, due to its high tensile and yield strengths.

The new alloy may be compounded by any of the methods used for melting and alloying metals with magnesium, such as by adding the palladium to a bath of molten magnesium which is preferably protected from oxidation by suitable flux.

I claim:

1. A magnesium base alloy containing from

0.01 to 3.0 per cent palladium, the balance being magnesium.

2. A magnesium base alloy containing from 0.1 to 2.0 per cent palladium, the balance being magnesium.

3. A magnesium base alloy containing 0.3 per cent of palladium, the balance being magnesium.

4. A magnesium base alloy containing from 0.01 to 3 per cent of palladium and characterized by a substantial improvement in at least one of the properties ductility, tensile strength, and yield strength as compared with magnesium without the palladium.

JOHN C. McDONALD.